# EUROPEAN PATENT APPLICATION

(11) **EP 0 055 492 A1**
(43) Date of publication of application: **07.07.1982**
(21) Application number: 81110846.3
(22) Date of filing: 30.12.1981
(51) Int. Cl.: C10M 11/00

(54) **A process for reclaiming used motor oil**

(30) Priority: 31.12.1980 US 221879
(71) Applicant: PHILLIPS PETROLEUM COMPANY, Bartlesville Oklahoma 74004 (US)
(72) Inventor: Classen, Theodore Michael, Bartlesville Oklahoma 74003 (US); Low, Jim Yuen-Fong, Bartlesville Oklahoma 74003 (US); Pahl, Robert Harold, Bartlesville Oklahoma 74003 (US)
(74) Representative: Dost, Wolfgang, Dr.rer.nat., Dipl.-Chem.

(57) **Abstract**

A process of recycling motor oil is provided wherein used oil is subjected to solvent extraction and the hydrocarbon extract is hydrogenated to produce a high quality stock.

## Description

The invention is concerned with a process for refining used lubricating oil. The used oil is subjected to solvent extraction to obtain a paraffin-rich phase, hydrogenation to eliminate unsaturated contaminants therein, and separation of the solvent to yield a high quality stock.

### Background

Motor oils are lubricants produced from petroleum by conventional refining techniques. They consist of a complex mixture of paraffinic hydrocarbons whose structures and properties render the mixture effective as a lubricant for internal combustion engines and the like. Besides hydrocarbon mixtures, motor oils often contain up to 30% by weight of additives such as detergents, pour point depressants, stabilizers, and viscosity modifiers. These oils break down during prolonged use, particularly at high temperatures, leaving various contaminants.

During use in an engine, the motor oil becomes contaminated with various impurities such as carbon, grit, ash, gasoline, water, -metal particles, particularly heavy metal residues, and other residues. Resins, oxidation products and unsaturated impurities can also be formed.

In the past, most used motor oil has been discarded or directed to low grade uses such as road oil or blending with heavy fuel oils. With increasing interest in fuel conservation, greater use is being made of motor oil reclaiming _{F}rocesses which can offer means for recovery of most of this premium hydrocarbon resource. Many of these processes have disadvantages such as a multiplicity of steps, high capital investment, waste disposal problems and low product recovery.

### Objects of the Invention

It is an object of this invention to provide a method for treating oil which has been drained from the crankcase of an internal combustion engine after residence therein during the engine's use.

It is an another object of this invention to provide a process for reclaiming motor oil wherein used oil is subjected to solvent extraction:
It is a further object of the invention to provide a method of reclaiming motor oil wherein the used oil is subjected to solvent extraction and the hydrocarbon extract is then subjected to a hydrogenation.

It is still another object of the invention to provide a process of reclaiming used oils wherein the used oils are subjected to solvent extraction, the hydrocarbon extract is hydrotreated, and the solvent from the extraction step is recycled.

### Description of the Invention

In one embodiment of the invention motor oil is reclaimed by a process which comprises the steps of:
(a) contacting used motor oil with one or more organic solvents under supercritical conditions of temperature and pressure so as to produce an extract phase;
(b) separating some or all of the extract phase from the other products of step (a);
(c) hydrogenating the extract phase from step (b);
(d) removing organic solvent from the extract phase before or after step (c); and
(e) recovering a hydrogenated oil product. The extract phase can usually also be characterized as an oil rich phase.

Optionally, the used oil feed may be processed through a flash separation or other separation device to remove impurities such as metals, water and/or gasoline components.

The oil feed may be combined with a portion or all of the solvent; preheated to extraction conditions; held for a suitable period of time to effect dissolution of oil thereby producing a solvent-containing extract which is relatively free of contaminants; passedthrough a separation zone such as a cyclone, filter, or phase separator to remove solids, part or all of the solvent, and/or undissolved residue; and the vapor phase introduced to a catalytic hydrotreater along with hydrogen. If desired, the temperature of the oil stream can be adjusted before hydroteatment, Hydrotrcater effluent is expanded and optionally cooled to condense refined oil which is removed from the system at the flash separator, Separator vapor is cooled and condensed to recover liquid solvent which can be recycled to the extraction step and hydrogen gas which may be recompressed and recycled to the hydrotreater,

The following ranges for process variables are suggested:

Solvents suitable for the supercritical extraction include single ring aromatics having not more than 3 carbon atoms on substituent groups, alicyclic hydrocarbons having at least 5 but less than 10 carbon atoms and acyclic hydrocarbons having at least 3 but not more than 10 carbon atoms- preferably C₃-C₇n-alkanes. Mixed solvents can also be used.

By "hydrogenation" or "hydrotreating" is meant addition hydrogenation, which is the reaction of hydrogen with non-aromatic unsaturation to produce a saturated product. Well-known catalysts are conventionally employed. "Hydrogenation" reactions are distinct from "hydrogenolysis" or destructive hydrogenation reactions which cause the rupture of the bonds of organic compounds and the subsequent reaction of hydrogen with the resultant fragments. A discussion of this distinction may be found in Condensed Chemical Dictionary, 9th Edition (1977).

The hydrogenation or hydrotreating step is conventional except for the presence of supercritical solvent which passes through unscathed unless it is aromatic, in which event a small fraction may be hydrogenated. Suitable catalysts useful in this step included those utilizing Group VIB and Group VIII metals or combinations thereof using a refractory support. Conventional hydrodesulfurizer conditions can be used. Suitable hydrode- sulfurization processes are disclosed in U.S. Patents 3,770,619 and 4,110,205. It is preferred to operate the hydrodesulfurizer at about the same pressure as the extraction step. In some cases, these two operations can be carried out at about the same temperature, but the temperature can be adjusted for hydrotreating.

The oil product from the process is a quality hydrocarbon base stock. It is believed to be equivalent to any virgin or unused hydrocarbon stock. Accordinclv. it can be mixed with conventional additives and subjected to conventional treatment to render it more useful as a lubricating oil.

### EXAMPLE 1

Used motor oil and n-heptane solvent were pumped into a nitro- gcn-pressurized one liter extraction vessel maintained at about 300°C and 750 psig (5.26 MPa). Pumping rate was about 10 ml/min for each fluid, and the fluids were preheated to about 300°C before introduction into the reactor. After approximately 15 minutes, product take-off commenced while pumping of both fluids continued at the same rate until 550 ml of n-heptane and 503 ml of oil had been added. Introduction of used oil was then discontinued, but pumping of n-heptane solvent continued at 10 ml/min for another 2½ hours to purge out the extracted oil. Product from the extraction was condensed and recovered. An analysis is given in the table following Example II.

### EXAMPLE III

A similar run was made using n-pentane solvent at extraction conditions of 225°C and 750 psig (5.26 MPa). An analysis is given below.

High percentages of the feedstock's ash content remained in the residue. In Example 1, for each 100 parts of feedstock, the total ash content was (7.4 x 2684) = 1.99 plus (92.6 x .0104) = 0.96, or 2.95 parts total ash. Since 1.99 parts ash was in the residue the percentage in the residue was ( )= 68%.

Likewise, for Example II, each 100 parts of feedstock contained (14.5 ×.216) = 3.13 plus (85.5 x 0.91) = 0.78, or 3.91 parts tctal ash. Since 3.13 parts ash remained in the residue( )= 80% of the ash remain- ed in the residue.

Both of the above examples demonstrate that high percentages of ash remain in the residue.

Reasonable variations which will become apparent to those skilled in the art can be made in the present invention without departing from its spirit and scope.

## Claims

1. A process for reclaiming used motor oil characterized by the steps of:
(a) contacting the used motor oil with at least one organic solvent under supercritical conditions of temperature and pressure so as to produce an extract phase;
(b) separating extract phase as an oil-rich phase from the other products of step (a);
(c) hydrogenating the extract phase from step (b);
(d) removing organic solvent from the extract phase, before or after step (c); and
(e) recovering a hydrogenated oil product.

2. The process of claim 1 characterized by including the further step of recycling the solvent removed in step (d) back to the reaction zone for step (a).

3. The process of claim 1 or 2 characterized in that the separation of the oil-rich phase is carried out by cyclone separation.

4. The process of claim 1 or 2 characterized in that step (d) is carried out by flashing.

5. The process according to at least one of the preceding claims characterized in that the organic solvent employed in step (a) is at least one member selected from single ring aromatic compounds having up to 3 carbon atoms on substituent groups, alicyclic hydrocarbons having from 5 to 10 carbon atoms, and acyclic hydrocarbons having from 3 to 10 carbon atoms.

6. The process of.claim 5 characterized in that the organic solvent employed is an alkane containing from 3 to 7 carbon atoms.
